

# UNITED STATES PATENT OFFICE.

JAMES L. COKER, JR., OF HARTSVILLE, SOUTH CAROLINA.

## PROCESS OF MAKING PAPER-PULP.

No. 830,570.

Specification of Letters Patent.

Patented Sept. 11, 1906.

Application filed December 18, 1905. Serial No. 292,359.

*To all whom it may concern:*

Be it known that I, JAMES LIDE COKER, Jr., of Hartsville, in the county of Darlington and State of South Carolina, have invented a new and useful Improvement in the Process of Making Paper-Pulp, of which the following is a specification.

The object of my invention is to utilize for paper-pulp-making purposes the ordinary timber pines which are found in very large quantities in the southern part of the United States, the principal varieties of which are known as "long-leaf" pine, (*Pinus palustris*), "short-leaf" pine, (*Pinus echinata*), "loblolly-pine," (*Pinus taeda*), and "Cuban" pine, (*Pinus heterophylla*). The wood of these Southern pines is very rich in resinous matter and substantially all of this matter must be removed from the wood before a good article of wood-pulp can be produced therefrom. Attempts, more or less successful, have been made to remove this resinous matter from the wood; but so far as I am informed all processes hitherto employed to obtain this result have depended upon the use of chemicals and have involved such expense as to be practically prohibitive in actual commercial manufacture. It is my object to effect this result simply, cheaply, and without the use of chemicals, and this result I attain by a process involving the steps of killing the tree, subjecting it with the bark on to the action of local natural agencies, whereby the resinous matter therein is changed, modified, or brought to such condition as to be innocuous in pulp making, removing the bark and cutting up and splitting the stripped timber into suitable lengths to arrest further deterioration of fiber, and then after removing the heart-wood from the sap-wood subjecting the thus-prepared sap-wood to any ordinary or suitable wood-pulp process. These are the steps which I have followed in practice with the result that in making paper-pulp from the thus prepared sap-wood none of the objectionable manifestations attendant upon the presence of resinous matter in wood is noticeable, and the pulp itself is of a quality that can only be obtained in the practically complete absence of resinous matter.

My invention is based upon the discovery, which I believe to be new with me, that if the killed pine tree be allowed to remain with the bark on exposed to the elements or to the action of natural agencies for a con-

siderable period of time; say from four to twelve months or even longer, the resinous constituents of the tree will by that time be changed and brought into such condition as to be practically innocuous for paper-pulp-making purposes. The length of time of exposure will vary with the season and with the character of the particular tree. The best time to kill the tree (whether by girdling or by felling) is in the early summer when the sap is circulating freely, since under these conditions the change in the resinous constituents proceeds more rapidly than at other times, although the same change will eventually but more slowly take place if the tree be killed at any other time of the year. The bark is allowed to remain on during the process of change for the reason that as I have found if the bark be removed from the green wood the direct exposure of the latter to the air seems to harden the resinous matter in the outer portion of the trunk, so that in quite a thick circumferential layer of the wood the resin remains practically unchanged, thus destroying the value of this portion of the wood for pulp making and retarding the change in the inner portion of the trunk.

The exact nature of the chemical change which takes place in the resinous constituents of the wood is as yet undetermined and is still under investigation; but it is not difficult to determine when that change, whatever it may be, has taken place. A simple test is to make an incision in the tree with an ax. If the tree is in proper condition and the change has taken place, the liquid which follows the blow will be limpid, non-viscous, and as fluid as water, almost tasteless, and with an odor which is ethery rather than resinous. As soon as this stage has been reached further decomposition or change should be stopped, because the wood itself by this time has materially depreciated in value by incipient decay both for fuel and for lumber, and further exposure will depreciate its value for pulp making also. To arrest further change, I strip the bark from the trunk and cut up the latter into convenient lengths and split these lengths so as to expose the interior. The heart-wood which occupies the interior of the tree still holds its resinous constituents in hardened condition and practically unchanged, and it therefore must be separated and removed from the sap-wood which forms the exterior portion

of the tree and in which the change in resinous constituents has been effected.

The sap-wood after its separation from the heart-wood is ready for immediate use as a 5 pulp-producing material or it may be stored for future use.

Having described my invention and the best way now known to me of carrying the same into effect, what I claim herein as new, 10 and desire to secure by Letters Patent, is as follows:

1. The improvement in the art of making pulp from the wood of the Southern pine, which consists in killing the tree, subjecting 15 it, with its bark still on, to the action of natural agencies, whereby its resinous constituents are modified or changed or brought to such condition as to be innocuous in pulp making, then, when tests show the tree has 20 been brought to this condition, removing the bark and cutting up and splitting the stripped trunk into suitable lengths, sepa-

rating and removing the core or heart-wood from the sap-wood; and finally submitting the thus prepared sap-wood to a pulp-making process, substantially as and for the purposes hereinbefore set forth. 25

2. In the art of making pulp from the wood of the Southern pine, the preliminary treatment of the wood for this purpose, 30 which consists in subjecting the killed tree, with the bark on, to the action of natural agencies until the trunk will yield a liquid having substantially the characteristics specified, and then stripping the bark from 35 the trunk and cutting up the stripped trunk into suitable subdivisions, substantially as and for the purposes hereinbefore set forth.

In testimony whereof I affix my signature in presence of two witnesses.

JAMES L. COKER, JR.

Witnesses:

W. LEE HELMS,  
PAUL E. JOHNSON.